

Patented May 4, 1926.

1,583,717

# UNITED STATES PATENT OFFICE.

EMIL HUBERT, OTTO LEUCHS, AND LUDWIG LOCK, OF ELBERFELD, GERMANY, AS  
SIGNORS TO FARBFENFABRIKEN VORM. FRIEDR. BAYER AND CO., OF LEVER-  
KUSEN, NEAR COLOGNE-ON-THE-RHINE, GERMANY.

## PROCESS FOR THE PREPARATION OF THREADS FROM CELLULOSE ACETATE.

No Drawing.

Application filed July 14, 1924. Serial No. 725,980.

To all whom it may concern:

- Be it known that we, EMIL HUBERT, OTTO LEUCHS, and LUDWIG LOCK, citizens of Germany, residing at Elberfeld, in the State of Prussia, Germany, have invented new and useful Improvements in a Process for the Preparation of Threads from Cellulose Acetate, of which the following is a specification.
- 10 In German Patent No. 274,260 a process is described, according to which a solution of acidyl cellulose is formed into threads by spinning into a highly concentrated salt solution. The fineness of the threads obtained according to this process depends 15 principally on the diameter of the jet and on the content of solid substance in the spinning solution, as the formed thread is completely coagulated very soon after leaving the jet and ceases to be extensible any longer. Thus, for instance, in order to obtain threads of an average capillary value of 7-8 deniers, it is necessary to work with very fine jets; in the most favorable case a jet 20 diameter of 0.2 mm. will be possible. With larger jet apertures, e.g. 0.4-1.0 mm., merely artificial horse-hair can be produced. In regard to the extraordinarily high viscosity of the spinning solutions of acidyl celluloses, 25 this circumstance implies very troublesome manufacturing difficulties amongst other things, it becomes necessary to work with very high pressures.
- 30 The noteworthy observation has now been made, according to which stretching spinning may be carried out in such a way that threads of a fineness of 3 deniers and less may be obtained from jets of about 0.6 mm. diameter, by using instead of a single solvent mixtures of the same.

To a solution of cellulose acetate in acetone, which is to be spun into a bath of concentrated calcium chloride solution, may be added for example benzene-alcohol, benzene-chlorobenzene, ethyl acetate, pyridine, chloro-alcohol, aniline etc. in quantities from 5-20 per cent. To an acetic acid solution which is to be precipitated with a concentrated solution of sodium acetate, may be added for example, chloroalcohol, acetylene tetrachloride etc. Very small quantities of these additions are sufficient for producing the desired effect.

As regards the choice of the substance to

be added, it is an important consideration 55 that the substance in question must be more difficultly extracted by the spinning bath, in consequence of which the coagulation of the thread is retarded. Moreover the addition must be adjusted according to the nature, concentration, and temperature of the spinning bath and to the length of immersion in the bath. Spinning may also be carried out, so that only a part of the solvent mixture passes into the spinning bath, while 60 the remainder evaporates on passing through the air. By this means special effects are produced in respect to lustre, strength and affinity for dyeing. According to these directions it becomes merely a matter of trial, 65 to find the best addition and the most suitable conditions for spinning.

The use of mixtures of solvents and precipitants or non-solvents is described in 70 French Patent No. 426,436, for example, the addition of alcohol, carbon tetrachloride, etc., to acetone solutions. There the object of this addition is to bring the spinning solution near to precipitation and to completely 75 coagulate the thread in the spinning bath by the addition of non-solvent to the spinning solution immediately after the thread leaves the jet. The new process surprisingly achieves the very opposite: the coagulation 80 of the thread is retarded which enables stretching spinning. This technical advance is obtained contrary to the direction of the French specification by adding the non-solvent to the spinning solution only in small 85 quantities.

In order to illustrate the new process more fully the following examples are given:

Example 1.—4 parts by weight of pyridine are added to 20 parts by weight of cellulose acetate dissolved in 78 parts by weight of acetone. Spinning at a temperature of 45° with a speed of spinning of 40 metres and using a spinning bath containing 23 per cent of  $\text{CaCl}_2$ . A capillary thread of 13  $\mu$  diameter corresponding to a titer of less than 3 deniers is obtained when jets of 0.7 mm. diameter are employed using a pressure of  $\frac{1}{3}$  atmosphere.

Example 2.—20 parts by weight of cellulose acetate are dissolved in 75 parts by weight of acetone and 5 parts by weight of chlorobenzene are added. The solution thus

obtained is spun into a calcium chloride bath of 23 per cent strength at a temperature of 42°. The calcium chloride spinning bath contains about 5 per cent of acetone calculated on the amount of calcium chloride solution. With a jet of 0.6 mm. diameter and employing a pressure of 1.2 atmospheres and a speed of spinning of 35 metres a monofil thread is obtained of a titer of 2.7 10 deniers.

We claim:—

1. Process for the preparation of threads of cellulose acetate which comprises spinning a solution of cellulose acetate into a 15 strong salt solution, said solution of cellulose acetate consisting of cellulose acetate and a single solvent therefor and one or more materials different from said solvent which are absorbed by the salt solution more difficultly than said solvent.
2. Process for the preparation of threads from cellulose acetate which comprises spinning a solution of cellulose acetate into a 20

strong salt solution, said solution of cellulose acetate consisting of cellulose acetate 25 and a single solvent therefor and pyridine, which is absorbed by the strong salt solution more difficultly than said solvent.

3. Process for the preparation of threads from cellulose acetate which comprises spinning a solution of cellulose acetate in acetone into a strong calcium chloride solution, said solution of cellulose acetate containing one or more materials different from acetone which are absorbed by the calcium chloride 30 solution more difficultly than the acetone.

4. Process for the preparation of threads from cellulose acetate which comprises spinning a solution of cellulose acetate in acetone containing pyridine into a strong calcium 40 chloride solution.

In testimony we have hereunto set our hands.

EMIL HUBERT.  
OTTO LEUCHS.  
LUDWIG LOCK.